

Nov. 28, 1939.

H. M. GERSMAN

2,181,228

METHOD FOR PRODUCING SLITTED BLANKS

Original Filed Aug. 14, 1933

2 Sheets-Sheet 1

*Fig. 1.*



*Fig. 2.*

INVENTOR  
Harvey M. Gersman  
BY *Pope & Powers*  
ATTORNEYS

Nov. 28, 1939.

H. M. GERSMAN

2,181,228

METHOD FOR PRODUCING SLITTED BLANKS

Original Filed Aug. 14, 1933 2 Sheets-Sheet 2



Fig. 3.



Fig. 4.



Fig. 5.



Fig. 6.



Fig. 7.

Fig. 8.



INVENTOR  
Harvey M. Gersman  
BY  
P&P Powers  
ATTORNEYS

## UNITED STATES PATENT OFFICE

2,181,228

## METHOD FOR PRODUCING SLITTED BLANKS

Harvey M. Gersman, New York, N. Y., assignor to Ferrex Corporation, New York, N. Y., a corporation of Delaware

Substitute for abandoned application Serial No. 685,017, August 14, 1933. This application April 21, 1939, Serial No. 269,264

4 Claims. (Cl. 80—60)

This application is a substitute for application No. 685,017 filed August 14, 1933.

This invention relates to the production of slitted blanks which are suitable for the manufacture of metal lath. More particularly the invention is concerned with the production of such blanks directly from stock of sheet bar or equivalent gauge.

Heretofore slitted blanks of the type generally described have been produced in a cold slitting operation, the sheets employed being produced in a hot rolling operation by so-called sheet mills. The latter, in order to meet different trade requirements are designed to produce a wide range of sizes and gauges. The units of the mill are, therefore, relatively large with respect to the particular requirements for the reduction of sheets suitable for the manufacture of lath, the rolls of the units usually being from 24 inches to 36 inches in length, whereas the sheets to be rolled are ordinarily from 8 inches to 10 inches in width. A certain part of the total cost of operating a mill is substantially constant regardless of the weight of the sheets being rolled, such part of the operating cost being dependent, among other factors, upon the size of the mill. It will be apparent, therefore, that in the case of light weight sheets such as, for example, are of the size required for the manufacture of metal lath the fixed part of the operating cost is so high with respect to the weight of the blanks produced as to be prohibitive. For this reason it has been the practice to roll the sheets in multiple widths in the sheet mills and then slit them into blanks of the desired size, the sheets being annealed and pickled to render them relatively soft and substantially free from scale in order to avoid injury to the slitting rolls and at the same time maintain at a minimum the power required in the slitting operations. The procedure described is laborious and costly.

The principal object of the present invention is to overcome the above objections, this object contemplating a novel process for the production of blanks of the type generally described which is simple, rapid and economical.

A further object is to provide for the production of blanks in such a manner that, with respect to a particular mesh or size openings, length and width, lath of various weights may be produced from the same gauge stock.

A further object is to provide a novel design of slitting rolls, this object contemplating the use of the said rolls to effect the final reduction of

the blank during, and as a part of, the slitting operation.

The invention is illustrated in the accompanying drawings, in which:

Figure 1 is a view in elevation of equipment for practicing the invention.

Figure 2 is a plan view of the equipment.

Figure 3 is an enlarged fragmentary section of the slitting and reducing rolls and is taken along line 3—3 of Figure 2.

Figure 4 is an enlarged fragmentary section of the slitting and reducing rolls taken along the line at which the sheet is initially engaged by the rolls.

Figure 5 is a similar view of the rolls along a line at which the slitting operation is complete.

Figure 6 is a similar view of the rolls along a line at which the reducing operation is complete.

Figure 7 is a similar view of the rolls, the section being taken through the clearances which provide the bonds by which the adjacent strands are connected.

Figure 8 is an enlarged fragmentary section illustrating slitting and reducing rolls of a modified form.

Figure 9 is a further modified form of slitting and reducing rolls, the rolls in this embodiment co-operating to reduce the thickness of the blank to final gauge during the slitting operation.

In accordance with the invention a heated sheet of stock of sheet bar or equivalent gauge is reduced to final gauge by reducing rolls, the sheet being slit during and as a part of the reduction operation. As illustrated, the equipment for accomplishing this includes a plurality of roll stands 10 through which the sheet is successively passed to effect successive reductions, the sheet being delivered from the last of the stands 10 to a final stand 11 in which its final reduction is effected and in which it is slit to provide strands and connecting bonds. The stands 10 and their rolls 12 provide in effect small reducing units, the said units being designed so that the light lath gauges are the base sizes, that is to say, the rolls 12 are designed for the reduction of sheets of narrow widths such as, for example, 8 inches to 10 inches. The rolls, therefore, are relatively stiff and can effect large reductions in such pass.

Hence the number of stands required is correspondingly small. As a result of this, and the fact that the sheets to be rolled are relatively short, the mill is compact and the sheets when heated can be reduced to final gauge and slit without requiring reheating. In this connection it is noted that the scale which forms upon the

sheets during the rolling operations hardens as the sheets cool, the critical value being in the neighborhood of 1300°. At a temperature lower than this the scale hardens to such a degree that 5 injury to the slitting rolls would likely result unless the sheet were first pickled. The invention, therefore, contemplates the slitting of the sheets while their temperature is above the critical value in order to avoid the necessity of pickling them. 10 Slitting the sheets while hot has the further advantage that the necessity of annealing them is also avoided.

Each of the rolls 13 of the stand 11 is made up of a series of discs 14 which are suitably secured upon a shaft 15. The discs are formed or provided with hub-like portions 16 which carry annular ribs 17. The hubs of the discs are secured against one another and their peripheries co-operate with the side walls of the ribs to provide annular recesses 18, it being noted that the discs are secured upon the shafts of the rolls in such a manner that the ribs of one roll are directly opposite and coincide with the recesses provided by the discs of the companion roll. In 20 other words, the ribs and recesses of one roll coincide respectively with the recesses and ribs of the other roll, the ribs of each roll working in the recesses of the other.

The ribs 17 are formed for a part of their depth 30 with parallel wall portions 19 which provide shearing edges and which co-operate with one another to slit the sheets into strands and connecting bonds, the depth of said portions preferably being just enough to insure a proper shearing action. From the parallel portions 19, the walls of the recesses taper as indicated at 20 toward the bottom walls 20a thereof. The degree of taper is determined by the extent to which the strands are to be elongated, the greater the degree of elongation desired, the greater the degree of taper that 40 is required. In any event regardless of the minimum degree of taper actually required to produce the desired amount of elongation the side walls of the recesses are preferably tapered to such a degree as to facilitate stripping of the sheets from 45 the rolls.

As a sheet 22 enters the rolls 13 parallel portions thereof are engaged by the ribs 17 and are displaced in opposite directions, the displaced portions entering the recesses 18. As best shown in 50 Figure 7 the ribs 17 are cut away at regular intervals as at 21 to provide bonds 23 for connecting the strands of the blank. The said recesses, as illustrated, are formed in co-operating pairs 55 which are arranged in staggered or break-joint relation, it being understood that if desired the connecting bonds may be provided by suitably notching only one of the rolls. The sheet which enters the rolls 13 is preferably of a temperature of the order of 1300° and is, therefore, relatively 60 plastic. Hence the initial action of the rolls is a forming action, that is to say the metal is forced into the opposite recesses of the rolls. Thereafter the shearing of the metal connecting the displaced 65 portions takes place and the strands are completed. As the displaced portions are forced into the recesses the tapered walls 20 thereof displace metal from the sides of the strands and as the 70 depth of the pass provided by the ribs and recesses is such that an increase in the thickness of the strands is prevented, the displaced metal is taken up solely by the elongation of the strands, the degree of such elongation, as indicated, depending upon the degree of taper of the walls 20.

75 In the embodiment illustrated in Figure 5 the

engaged portions of the blank enter those parts of the recesses which are defined by the wall portions 20 before the slits which delimit the engaged portions are completely formed. The elongation of the strands therefore, being before the latter are 5 completely defined. In this embodiment the depth of the pass, that is to say the distance between the peripheries of the ribs and the bottom walls of the recesses, is equal to the thickness of the sheet at the time it enters the rolls. It will be 10 apparent, therefore, that in such case the thickness of the sheet remains the same during its passage through the rolls, the elongation of the strands being effected solely by the displacement 15 of metal from their sides. It is preferred, however, that the sheet be reduced to final gauge or thickness in the slitting rolls. To this end the rolls 13a of the embodiment shown in Figure 9 are associated in such a manner that the ribs and 20 recesses 17a and 18a, respectively, thereof co-operate to provide passes which are less in depth than the thickness of the sheets which are delivered to the rolls from the adjacent stand 10. In this embodiment the passes provided by the ribs and recesses are filled before completion of the 25 slitting operation, the strands being reduced in thickness as the metal defining the strands is severed. It will be apparent, therefore, that in this embodiment the elongation of the strands is 30 effected not only by displacing metal from the sides of the strands but also by reducing them in thickness.

As the slitted sheets emerge from the slitting rolls they may be formed in packs or coils and 35 covered. At this time they still retain sufficient heat to self-anneal themselves to a point at which they will be soft enough for the subsequent expanding operation, it being unnecessary for the sheets to be as soft for expanding as for shearing.

It will be noted that the depth of the ribs 16 is 40 substantially less than their width. This has the advantage that the heat which is transferred to the ribs from the sheets will be distributed over a relatively large area and hence will be quickly dissipated. Warping of the ribs, therefore, is 45 avoided. As only a small part of the strand forming operation is actually shearing and that of hot metal, the shearing edges of the ribs will operate effectively over long periods of time.

The embodiment illustrated in Figure 8 includes 50 companion rolls 13b which are formed with co-operating ribs and recesses 17b and 18b respectively. In this embodiment the tapered side walls 20b of the ribs are curved instead of straight, the rolls in other respects being substantially the 55 same and functioning in substantially the same manner as those shown in Figure 4.

From the foregoing it will be apparent that 60 slitted blanks of final gauge may be produced directly from stock of sheet bar or equivalent gauge. The elongation of the strands in the manner described has the advantage that with respect to expanded sheets of a particular size various weights of sheets may be produced from stock 65 of the same gauge. In other words, the weight of the expanded sheets may be decreased by increasing the amount of reduction of the strands while the weight of the expanded sheets may be decreased by decreasing the elongation of the 70 strands, it being understood that in each case the length of the sheet bar is determined by the weight of the finished sheet. Slitted blanks of the required size and weight may, therefore, be produced from one, or at the most, two gauges 75

of stock. As the mill is designed with particular reference to the reduction of stock of a particular gauge the operating costs thereof can be maintained at a minimum.

5. While the slitting and reducing rolls 13 are shown as comprising gangs of discs it is to be understood this is for purposes of illustration only. They may, for example, be formed from solid rolls, the co-operating ribs and recesses in 10 this case being formed by a suitable milling operation.

I claim as my invention:

1. The method of producing a slitted blank suitable for the manufacture of metal lath which 15 includes heating the sheet from which the blank is to be formed, slitting the sheet to provide strands and connecting bonds by deflecting alternate parallel portions in one direction while deflecting the intermediate parallel portions in 20 the opposite direction, and displacing metal from the sides of said portions as they are deflected whereby to elongate the strands correspondingly.

2. The method of producing a slitted blank suitable for the manufacture of metal lath which 25 includes heating the sheet from which the blank is to be formed, slitting the sheet to provide strands and connecting bonds by deflecting al-

ternate parallel portions in one direction while deflecting the intermediate parallel portions in the opposite direction, and displacing metal from the sides only of said portions as they are deflected whereby to elongate the strands correspondingly. 5

3. The method of producing a blank suitable for the manufacture of metal lath which includes slitting the sheet from which the blank is to be formed by deflecting alternate parallel portions 10 in one direction while deflecting the intermediate parallel portions in the opposite direction, and rolling the said portions as they are deflected in the manner described whereby to elongate the strands. 15

4. The method of producing a slitted blank suitable for the manufacture of metal lath which consists in slitting the sheet from which the blank is to be formed to provide strands and connecting bonds by deflecting alternate parallel portions 20 in one direction while deflecting the intermediate parallel portions in the opposite direction, and displacing metal from the sides of said portions and reducing them in thickness as they are deflected whereby to elongate the strands corre- 25 spondingly.

HARVEY M. GERSMAN.